

April 18, 1933.

G. E. PELTON

1,904,628

INK TRANSFER MEMBER AND METHOD OF MAKING THE SAME

Filed May 5, 1927



INVENTOR.  
George E. Pelton  
by Parker & Brookins  
ATTORNEYS.

## UNITED STATES PATENT OFFICE

GEORGE E. PELTON, OF LOS ANGELES, CALIFORNIA, ASSIGNOR TO THE GEORGE E. PELTON COMPANY, A CORPORATION OF DELAWARE

## INK TRANSFER MEMBER AND METHOD OF MAKING THE SAME

Application filed May 5, 1927. Serial No. 189,180.

This invention relates to improvements in what are generally known as typewriter ribbons, and for convenience, such term will be hereinafter used in the description of the invention, altho it is, of course, to be interpreted broadly as including any of those reproducing instrumentalities in tape form adapted for use not only on typewriters but on various other kinds of machines, such as 5 adding machines, cash registers, time clocks, etc.; or, in other words, all kinds of printing mechanisms in which the ink is not applied directly to the impression means.

The invention is particularly adapted for 15 use with the new electrically operated typewriters which have recently been put on the market, the operation of which puts a terrific strain on the ribbon. This is especially noticeable upon the edges of the ribbon. While 20 such electrically operated machines greatly relieve the typist, they materially increase the strain and wear upon the ribbon. The lightest feather touch of the typist's fingers, when making sixteen or more carbon copies 25 simultaneously, brings into operation an electric motor which causes the type to strike against the ribbon's front surface or the surface towards the type with a force many times greater than with any hand operated 30 typewriting machines. Such very severe blows quickly injure the threads of prior fabrics and especially the edges of both woven and glued edge ribbons. It may also be noted that with the old style of typewriting 35 machines, the type never closely engaged the edge of a relatively wide ribbon formerly used, and there was little or no force tending to wear the threads very thin and stretch or cut them like the force of an electric 40 typewriter which drives the type bars equipped with very small sharp edged type such as the micro or elite type. Such type faces require the use of very thin fabrics, and while the additional strength needed in 45 a ribbon for electric machines can be secured by using much thicker and stronger materials, yet such materials do not permit one to use small type. The modern typewriting machine also puts a very great strain upon 50 the ribbon's edge when shifting for capitals.

Take the Underwood as typical. The ribbon feeding mechanism is connected with the type actuating mechanism and in writing capital letters each type bar stroke lifts the ribbon high up above its normal position, and the 55 surface of the ribbons towards the type pulls tensely against the sharp edges of the ribbon guide.

Whether the edge is glued or woven, when 60 electric machines such as those above mentioned are employed, I find that when making many carbon copies simultaneously that the impact of the type against the threads of the ribbon is so great as to wear the threads thin, make them baggy and they sag and 65 wrinkle and curve in the machine instead of retaining their shape and lying flat in the machine as they must to give fine results.

It is therefore the primary object of my 70 invention to produce an inking ribbon capable of withstanding the severe wear to which such ribbons are subjected under modern conditions to the end that their useful life may be extended. I have attained this 75 object by applying to that face of the ribbon which will be struck by the type a tough, flexible wear-resisting coating of one of the cellulose esters, such as pyroxylin, and then inking the coated ribbon. Although the use 80 of such a coating tends to prevent unravelling along the edges I prefer to enclose the edges of the ribbon with a similar material.

Preferably I use as the fabric base of my 85 ribbon a specially woven silk material, not less than two thousandths of an inch thick and not more than six thousandths of an inch thick, according to the use and the machine which employs said material as an inked 90 ribbon for writing; both the warp and the filling are woven very closely of yarn that is pure, unadulterated silk of first quality and of very soft character. The closer the 95 weave of the warp and filling and the better the quality of the weaver's work, the better the results will be from the material when used as an inked ribbon because of the exacting requirements as to uniform thickness, absence of flaws or knots or tied threads, or 100 frayed or broken threads, when said mate-

rial is used in modern typewriters equipped with very small type. It is readily seen that a very minor imperfection in the weaver's results will blur a micro type impression or 5 an elite type impression. I prefer the material to be in not less than one thousand yard lengths and not less than forty-two inches in width. It is customary to use some 10 sizing or stiffening material in silk cloth which is to be slit and the edges glued and the material used in making inked ribbons for typewriters. This sizing or starch or 15 gum material which is used cuts down just that much the absorbing and ink retaining capacity of the silk threads and does this not only on the side the type strike against but also all thru the threads and on the side towards the writing paper. It is preferable 20 to use no sizing material whatever to stiffen the silk material, preparatory to slitting. The natural gum in the threads of silk must 25 of course be entirely removed or "boiled off", and the material may be finished in any suitable manner but must not be starched or sized if the best results are to be obtained later when the material receives its ink supply at the inked ribbon factory.

The silk material is wound by machinery 30 for that purpose upon a tube of suitable diameter and length and is then coated by means of a coating machine or other suitable equipment with a very thin layer of cellulose material and dried. The coating 35 should be done before any ink is applied because one cannot properly strengthen silk or other fibres which have a coating of ink on the surface or side to which the coating of cellulose or other reinforcing material is to 40 be applied. The ingredients in or composing the ink prevent a cellulose or other reinforcing coating material from adhering to same to an extent equal to that with which such coating material will adhere to the uninked 45 threads or fibres themselves.

The fabric may be narrow strips with woven edges, exactly the right width for use in the particular type of machine which is to use same as a vehicle for carrying ink 50 and as an inked ribbon for writing. In this case, of course, much smaller machines and equipment are used for coating the material. The present invention is not limited to woven edge inked ribbon material nor is it limited 55 to glued edge inked ribbons or ribbons which have been slit from wide goods by suitable slitting machines and the edge threads or raw ends fastened by some suitable adhesive.

I preferably use a wide web of silk material 60 which, after coating, is slit into ribbons of the desired width. The material feeds into the slitting machinery very much more efficiently than soft uncoated material and does not wrinkle and fold and curl, and there 65 will be little or no danger of having frayed

edges. By reason of the powerful coating material which has been applied the material has been reinforced and better withstands the tension and strain put upon it by the slitting and winding machinery. It is also true 70 that when coated the woven edge and glued edge ribbons have much greater tensile strength and are better able to withstand all strain put upon them by winding, inking, finishing and spooling equipment. I prefer 75 to slit the material before it is inked.

After being slit into the required widths, altho all of the threads have been fastened together and reinforced and greatly strengthened by the coating material, I prefer to 80 apply a strip of Dupont cellulose cement, or other suitable impervious cellulose or adhesive material, to the edges of the ribbons.

In prior silk ribbons it has been the practice to put a line of gum or other adhesive to simply close the raw ends and bind them to each other continuously. This gum or adhesive is pervious to ink and absorbs ink. Although my coating itself binds the edges 85 of the ribbon, I prefer to fill the rest of the absorbing capacity left in the opposite and uncoated sides of the edges with cellulose or other suitable cement or adhesive material. One of the principal reasons why I prefer to 90 use silk material of the specifications and characteristics mentioned above is that due to the uniform diameter of the threads and fibres, it is possible to apply a uniformly even coating of the cellulose or other material on one side of the ribbon, and it is also 95 possible to meet the very exacting, rigid requirements of modern typewriting machines which write along the edges of inked ribbons, because with silk edge threads the edging 100 material is applied uniformly and is absorbed uniformly not only as to the raw ends which are bound together but it enables one to perfectly and exactly bind the raw ends of the filling threads or crosswise threads to 105 the warp or lengthwise threads along the said edges, thereby greatly strengthening and reinforcing said edges to better meet the requirements of modern electric and other machines as set out above where the 110 type strike against the surface of the inked ribbon and where the type put a strain on the edge of the ribbon when the machine shifts for capital letters and also the strain 115 on the edge of the ribbon due to its rubbing 120 with tension upon the sharp metal edges and surfaces of the vibrator of the machine.

I prefer to not only put the strip of cellulose material to bind the raw ends together but also to entirely fill up the filling or crosswise threads where they come in contact with or touch or join or lap around the lengthwise or warp threads, and the warp threads, lying very close to the outer edges of the silk ribbon or other fibre material, are 125 completely saturated and loaded with suit-

able cellulose or other material and cemented or joined to the said crosswise threads on the side opposite to that which received the coating at first before the material was 5 slit into ribbons. This results in a ribbon that not only has all of its thread on one side covered by a powerful coating which reinforces and greatly strengthens said ribbon but also it results in a ribbon which 10 has its warp threads and filling threads and raw ends all joined together and the outer edge threads are further strengthened because said cellulose or other adhesive is in both surfaces of said threads binding said 15 threads together as to both sides of the ribbon for a slight distance in from each edge of said ribbons but also to said warp.

I prefer to now ink said ribbons and to apply the ink on the side opposite that which 20 was coated before the material was slit. If the ink applied is a thin ink or is similar to the inks used for making lightly inked typewriter ribbons, it may be applied on both sides of the fabric or silk material 25 by means of the usual ink rolls. As one side of the silk or other fabric material has already received a coating, very little ink will be absorbed on the coated side even though the material or fabric or silk base is passed 30 right through an ink container and through ink rolls which press out the surplus ink. Such a thin ink will be almost entirely in that part of the threads or fibres which have no coating and consequently even if applied 35 on both sides, there will be a very slight amount of ink coming in contact with the type.

The resultant ribbon now has its ink supply where it can be most efficiently given 40 out upon the writing paper, and said ink cannot be wasted by the type striking directly into the threads or fibres which in prior ribbons are saturated with ink and have as much ink to give out on the type 45 side as on the side towards the writing paper. By reason of the cellulose coating on the one surface of the ribbon which the type strike against, the type cannot strike directly into the threads or fibres of silk or other 50 material, thus picking up fibres to clog and fill the type. By reason of said ribbon material being greatly strengthened and reinforced as set out above, it lies flat in the machine, retains its shape, the threads do not 55 wear thin and become roughened and ragged in appearance and under the most severe pounding of small metal type in electric machines making many carbon copies simultaneously said ribbon material is in good 60 condition after being reinked and used a second time. The coating which I employ does not saturate the fabric and thus impair the ink-carrying capacity of the ribbon, nor does it react injuriously with the ink nor absorb moisture in damp weather.

The accompanying drawing shows by way of illustration how my invention may be applied to a typewriter ribbon, and this drawing is a fragmentary cross section of the ribbon greatly magnified, the middle portion of the ribbon being broken away. In this drawing A represents the fabric of the ribbon, one face of which has a coating B of a cellulose ester composition applied thereto; this face of the ribbon being the one which is struck by the type. C represents an impervious cellulose composition which impregnates the edge portions of the ribbon.

While I have described my invention as employing a base fabric of silk, it is to be understood, however, that cotton, artificial silk, ramie silk, paper, rubber, or combinations of any of these or even very thin strips of cellulose material, may be employed.

I have found that a pyroxylin solution is well adapted as the coating material but other materials having the same qualities such as kataloid acetate or other cellulose esters might be used.

Having thus described the invention, what is claimed as new and desired to be secured by Letters Patent is:

1. The method of making inking ribbons which comprises coating the face of a strip of closely woven, tight, compact, uninked fabric which is to be struck by the type, with a cellulose ester to form a coating of such character that it is securely attached to said uninked fabric without the use of any liquid cement or other foreign material and said coating not being sufficiently pervious to permit ink to be screened therethrough and transferred therethrough, and said coating not impregnating said fabric and not filling up the interstices of said fabric, and applying ink to the fabric and filling the fabric from face to face and into the coating and into the interstices of the fabric with ink, the coating being applied solely to the face of the fabric which is away from the writing surface and towards the type, and said coating being distinguished by the fact that it is dry and non-injurious to ink at the time the ink is applied to said coated fabric.

2. The method of making inking ribbons which comprises coating the face of a web of unsized, unstarched closely woven, tight, compact, uninked silk material which is to be struck by the type, with a cellulose ester without the use of any third material between said coating of cellulose ester and said silk material, and then slitting the web into ribbons of the desired width, and inking the ribbons.

3. The method of making inking ribbons which comprises coating one face of a strip of uninked fabric with a cellulose ester without the use of a third material between said coating and said uninked fabric, impregnating the edge portions of the ribbon with a cellulose ester impervious to ink, and then filling

the remaining portions of the fabric with ink and said coating is unfit for screening ink therethrough and is a wear-resisting coating for extending the life of the fabric material and said coating does not impregnate the base and does not fill the interstices of the fabric.

4. The method of making inking ribbons which comprises coating the face of a web of unsized, unstarched, closely woven, tight, compact, uninked silk material which is to be struck by the type with a cellulose ester, which is attached to the uninked silk material before any ink is applied to said silk and without the use of any third material such as liquid cement or any other foreign material between said cellulose ester coating and said silk, and said coating does not impregnate the silk material and does not fill the interstices of same, and then slitting the web into ribbons of the desired width, impregnating the edges of the ribbon with a cellulose ester impervious to ink, and then filling the remaining portions of the fabric with ink.

5. The method of making inking ribbons which comprises coating the face of a strip of closely woven, tight, compact, uninked fabric which is to be struck by the type with a cellulose ester which does not impregnate the base and does not fill the interstices of said base fabric and said coating is unfit for screening ink therethrough to the type faces but is expressly for increasing the wear of the fabric material, and said coating is applied to said fabric before any inking is done and then applying ink to both faces of the coated ribbon, filling the fabric with said ink and filling the interstices of said fabric with ink.

6. The method of making inking ribbons which comprises coating the face of a web of unsized, unstarched, closely woven, tight, compact, uninked silk material which is to be struck by the type with a cellulose ester, which does not impregnate the silk material and does not fill the interstices of said material and said coating is unfit for screening ink therethrough to the type faces but is expressly for the purpose of increasing the wear of the silk material, and said coating is applied to said silk before any inking is done, and slitting the web into ribbons of the desired width, impregnating the edges of the ribbon with a cellulose ester impervious to ink, and then applying ink to both faces of the coated ribbon, filling the silk material with said ink and filling the interstices of said silk material with ink.

7. The method of making ink transfer members which comprises superficially coating an uninked, closely woven, tight, compact, base material with a thin film of pyroxylin solution, sufficiently pervious to retain and contain at least one ingredient of the materials which make up and comprise ink but unfit for transferring ink therethrough and said pyroxylin solution being of such char-

acter as to form a powerful, wear-resisting, protective film and being on the side of the ink transfer member towards the type and being distinguished by its capacity to keep the ink from fouling the type, said coating being attached to the uninked base material and united to the surface of the base to form a flexible and tough impact-receiving surface, without impregnating the base and without filling the interstices thereof, no third material such as liquid cement or other foreign material being used in attaching said film or coating to said uninked base material, and said coating and base being thoroughly dried before inking so as to evaporate all solvent material in said coating or film, and then inking said base material, filling the fibers of said base from face to face but not through the coating to the outer face of the coating or film, and filling the interstices of the base with ink, the pyroxylin coating being applied solely on the face of the base toward the type, but the fibers of the base and the base, exclusive of the film or coating, being filled with ink.

8. The method of making ink transfer members, which comprises superficially coating one face of a closely woven, tight, compact, base material which contains no ink with a thin film composed of pyroxylin solution applied without penetrating the interstices of said base material so as to reduce the ink absorbency of said base material and without impregnating the base material with said pyroxylin solution, and said coating being unfit for ink to be transferred therethrough to the type faces, and drying said coating thoroughly before any inking is done to any portion of said base material, and when same is thoroughly dry and all solvents originally in said pyroxylin solution have been evaporated to an extent that the dry film cannot, when attached to said base material without the use of a third material such as liquid cement or other foreign material, injure the ink later applied to said base material, and then inking said base material by applying ink to the uncoated side which is away from the type and towards the writing surface and impregnating the base with ink and filling the interstices with ink and said ink extending from face to face of said base material and penetrating or being retained slightly by the surface of said film and at least one of the ingredients of said ink discoloring the outer surface of said film.

9. The method of making ink transfer members for use in typewriting and other printing machines which comprises applying a thin cellulose ester coating directly to an uninked base material comprising uninked, closely woven, compact, tight, silk fabric, free from starch, sizing and foreign materials which may reduce its ink-absorb-

ing capacity, and said cellulose ester coating being unfit for transferring ink therethrough, and so applied that when it is dry it cannot materially impair the ink-absorbing capacity of the fibres of said silk fabric, and said coating not filling the interstices of silk fabric and does not impregnate said silk fabric, and thoroughly drying said coating and then applying ink to the uncoated 10 face and filling the interstices of said silk fabric with ink and impregnating the silk fabric with ink and said cellulose ester material is of such character that it will permit at least one ingredient of a thin typewriter 15 ribbon ink to be retained on its surface to some extent permanently discoloring said surface along one face of boiled-off silk fabric free from starch, sizing and other foreign material, cutting said fabric into ribbons, 20 and thereafter inking said ribbons.

10. That improvement in the art of making silk inking ribbons comprising the use for that purpose of a very closely woven, tight, compact, uninked silk fabric base, and 25 boiling off said silk fabric base, and using no sizing and no finishing material and other foreign material in said uninked silk base in preparing the silk fabric for its cellulose coating, and applying a coating of a cellulose 30 ester material along one face of said uninked silk base, said cellulose ester coating being thoroughly dry and all solvents having been evaporated that might injure the ink later applied to said silk material, and said coating 35 being distinguished by its inability to transfer ink therethrough and said coating does not impregnate said silk material and does not fill up the interstices of said silk and does not materially impair the ink-absorbing 40 capacity of said silk fabric base material, and thereafter impregnating the absorbent fabric base so coated with a suitable ink.

11. That improvement in the art of making inking ribbons comprising applying a thin coating of a cellulose ester or analogous cellulose material over one face only of a sheet of uninked, compact, closely woven, tight, absorbent fabric previously freed 50 of natural gum and all foreign materials, and drying said coating thoroughly before applying ink to said coated fabric, and said coating being distinguished by the fact that it is unfit for transferring ink therethrough 55 and it does not impregnate said fabric and does not fill the interstices of said fabric and does not materially reduce the ink absorbing capacity of said fabric, and, after said coating is thoroughly dry and the solvents of 60 said cellulose ester coating material are evaporated to an extent that said coating cannot injure the ink later put into it, cutting the sheet into ribbons, and inking the coated ribbons thus produced on at least the 65 uncoated face thereof.

12. The method of making inking ribbons which comprises coating one face of a strip of closely woven, tight, compact, uninked fabric with a cellulose ester which does not impregnate the base and does not fill the 70 interstices of said base fabric and said coating is unfit for screening ink therethrough to the type faces but is expressly for increasing the wear of the fabric material, and said coating is applied to said fabric before any 75 inking is done and then applying ink to both faces of the coated ribbon filling the fabrics with said ink and filling the interstices of said fabric with ink.

13. The method of making inking ribbons 80 which comprises coating one face of an uninked paper base material with a cellulose ester and then impregnating the edge portions of the base with a cellulose ester impervious to ink said coating being unfit for screening ink therethrough and said coating does not impregnate said base nor fill the interstices of said base, and there is no third material such as liquid cement, gelatine or 85 an adhesive or other foreign material between said coating and said base material.

14. The method of making ink transfer members which comprises applying a cellulose ester material to one face only of a closely woven, tight, compact uninked base material, which contains no liquid cement and no gelatine and no other foreign material, and no ink, and allowing the solvents in the cellulose ester material to dry and to evaporate, and forming a coating on the one face 95 of the base which does not impregnate the base and does not fill the interstices of the base and which is unfit for passing ink therethrough, and then inking said base material and impregnating the base with ink and filling the interstices of the base with ink, said coated face to be towards the type and no coating to be on the face away from the type, said face being filled only with ink.

15. The method of making ink transfer members which comprises making that face of an uninked absorbent base material of the character described, on the side towards the type, less absorbent than the face away from the type, which latter face is to have no coating of any kind and then inking said base material on at least the face towards the writing surface and filling the interstices of the base with ink and the face towards the type to be so non-absorbent that ink cannot be transferred thru same to the type faces but said face towards the type to be of such material and consistency that it is distinguished by its capacity to retain and contain at least one ingredient of a thin typewriter 100 ribbon ink on and in its surface, and winding said ink transfer member so that the base full of ink is in intimate contact with the face which goes towards the type.

16. An inking ribbon comprising a strip 105

- of fabric having an absorbent body portion carrying ink, and a coating of a cellulose ester on one face said coating being fastened to the uninked body portion without the use of any adhesive or liquid cement or other material between said coating and said body portion, said ribbon having the edges impregnated with a cellulose ester impervious to ink.
- 10 17. An inking ribbon comprising a strip of fabric having an absorbent ink-carrying body portion, a coating of a cellulose ester on one face, said coating being fastened to the uninked body portion without the use of any adhesive or liquid cement or other material between said coating and said body portion, and a binding of a cellulose ester saturating the edges of the fabric and rendering them non-ink absorbent.
- 15 18. An inking ribbon comprising a strip of fabric having an absorbent body portion impregnated with ink, a coating fastened to the uninked body portion without the use of any adhesive or liquid cement or other material between said coating and said body portion, said ribbon having its edges impregnated with a cellulose ester impervious to ink.
- 20 19. An ink transfer member comprising an absorbent, dry, uninked paper base, ink, a coating material, said paper base being coated on one face only with a cellulose ester secured to the uninked base material without the use of a third material between the base and said film or coating, and without penetrating the paper base sufficiently to materially reduce the ink-absorbing capacity thereof, said film being of sufficient density to prevent the passage of ink therethrough to an extent sufficient to supply ink to a writing surface, said film being applied to the side towards the type and away from the writing surface and said film being unfit for screening ink through to the type faces, and said base carrying ink in the interstices thereof and in the body portion of the base.
- 25 20. An inking ribbon comprising an absorbent body portion comprising fabric carrying ink and a coating of cellulose ester, which is sufficiently pervious to contain and retain on the surface of the coating at least one ingredient of the materials forming a thin typewriter ribbon ink, but said coating being of a composition and construction unfit for use as a screen for the passage of ink therethrough to the type faces and said coating being only suitable for use on the face of the ribbon struck by the type, and being applied to the base or fabric material prior to any inking of any portion of said base or fabric material and said coating and said base being a unit material firmly united without the use of any adhesive or liquid cement or other third material between said coating and said base or fabric material.
- 30 21. A typewriter ribbon comprising an absorbent combination of silk and cotton and having a face of the fabric coated with a wear resisting material pervious to ink without impairing the ink absorbing capacity of the remainder of the ribbon, and an ink supply absorbed by the fabric.
- 35 22. An inking ribbon comprising an absorbent body portion comprising fabric carrying a coating of a cellulose ester attached to the said fabric before any inking of the fabric which is slightly pervious to ink, on the face of the ribbon struck by the type, but unfit for screening ink therethrough, the edges of the ribbon being impregnated with a cellulose ester impervious to ink.
- 40 23. An inking ribbon comprising a strip of uninked fabric coated on one face only with a protective film of a cellulose ester applied directly to the fabric on the face thereof to be struck by the type without impregnating the fabric, said coated fabric having its edges impregnated with an impervious cellulose ester and the remaining portions of said fabric being filled with ink.
- 45 24. An inking ribbon comprising a strip of uninked fabric coated on one face only with a protective film of a cellulose ester applied directly to the fabric on the face thereof to be struck by the type without impregnating the fabric, said coated fabric having ink applied to both faces thereof.
- 50 25. An ink transfer member comprising an uninked, closely woven, tight, compact fabric base material, coated on one side with a superficial protective film of cellulose ester unfit for use as a screen to transfer ink therethrough to the type faces and said coating, extending into the fabric to a slight depth and united to the fibers of the fabric to form a flexible and tough type impact receiving surface without impairing the ink absorbing capacity of the opposite side of the ink transfer member, and an ink supply absorbed by the fabric, and said coating does not impregnate said fabric and does not fill up the interstices of said fabric and the fibres of the fabric are impregnated with ink and ink fills the interstices of the fabric and there is no third material used between the cellulose ester film or coating and the fabric base.
- 55 26. An ink transfer member comprising a fibrous base material coated with a superficial wear-resisting film of cellulose ester secured to the uninked base material without materially reducing the ink-absorbing capacity thereof, said film being of sufficient density to prevent the passage of ink therethrough to an extent sufficient to supply ink to a writing surface, said film being applied to the type side of said transfer member, and an ink supply absorbed by said base material.
- 60 27. A typewriter ribbon comprising an ab-

- sorbent combination of silk and cotton and having its edges impregnated with a cellulose ester impervious to ink.
28. An ink transfer member comprising a base fabric of absorbent silk and cotton in combination, said base being closely woven, tight, compact and uninked at the time it is coated with a cellulose ester material on the face towards the type, only, and said coating consisting of a material unfit for use as a screen to pass ink therethrough to the type faces and being expressly for increasing the wear resistance of said silk and cotton base material, and said coating does not impregnate said silk and cotton material and does not fill the interstices of same and there is no cellulose-coating on the face towards the writing surface but this face is full of ink and the silk and cotton are impregnated with ink and ink fills the interstices of said silk and cotton base, and there is no foreign material of any kind such as liquid cement, gelatine or an adhesive in between said coating and said silk and cotton base material, and said coating is thoroughly dry before it is inked in order that the ink may not be injured during the drying of the solvents and evaporation of solvents in the coating material which is on the face towards the type.
29. An ink transfer member comprising a compact paper base material, tightly and compactly fabricated and formed, coated on one face only with a powerful, protective film of a cellulose ester secured to the uninked paper base, and said film being composed of a material so non-porous as to be unfit for use as a screen to screen ink therethrough to the type faces and said film being of sufficient density to prevent the passage of ink therethrough to an extent sufficient to supply ink to a writing surface to make impressions that are legible, and said film being applied and fastened to the type side of said ink transfer member and being distinguished by the fact it does not impregnate the uninked paper base and does not fill the interstices of the base, and said film being thoroughly dry and noninjurious to the ink which is in said paper base and in the interstices of said paper base, penetrating through the body portion of said paper base but not through the outer face of said film.
30. An inking ribbon comprising a ribbon of absorbent fabricated fibrous material containing ink and having opposed face portions at one of which its ink supply is exposed, and the other one of which has a surface film or coating of a cellulose ester material adhering directly to said fibrous material or base material, said film being of sufficient density to prevent the passage of ink therethrough to an extent sufficient to transfer ink to a writing surface or to the type faces, said film being fastened or secured to said ribbon while uninked, and being only

suitable for use on the face of the ribbon struck by the type, and being of such character as not to materially impair the ink absorbing capacity of said ribbon or base and not to fill the interstices of same, and said absorbent ribbon or base material being impregnated with ink opposite said coating, and exclusive of said film or coating.

31. An ink transfer member comprising a body portion which is ink absorbent, a coating, and ink, and having its edges impregnated with a cellulose ester material impervious to ink, said coating being attached directly to said body portion before inking same.

32. An ink transfer member comprising an absorbent, compact, closely woven, tight base material, a coating, and ink, and having its edges impregnated with a cellulose ester material impervious to ink, and said coating being attached directly to said base before inking same, and said coating being expressly to extend the life of the base material and being on the face which is struck by the type.

33. An ink transfer member comprising an absorbent paper base, ink, and a coating material attached to the type face of said member as a superficial, overlying, superimposed coating which does not appreciably impair the absorbing capacity of said base, said coating being secured to the base before inking and without the use of a third material between the base and said coating, the type face of said base being more wear resisting than the writing surface face due to said wear resisting coating, and said coating being of such density as to prevent the screening of ink therethrough to the type, or to the writing surface if the member were reversed.

34. An inking ribbon comprising a ribbon of unadulterated silk fabric free from natural gum and composed of yarn of a soft character and said fabric being very closely, tightly and compactly woven and of high thread count in both warp and filling, and containing ink on both faces, but much less on the coated face, said ribbon having opposed face portions, one of which is exposed and the other of which has a thin coating of a cellulose ester material adhering directly to uninked surfaces of the threads of the fabric and said silk was uninked and no foreign material was placed between said silk and said coating at the time said cellulose ester was applied to the uninked silk fabric and said cellulose ester was dry at the time the silk fabric was inked and said coating is unfit to transfer ink therethru and it does not impregnate said base silk material and there is no cellulose coating on the face away from the type.

35. An ink transfer member comprising ink, an uninked absorbent, compactly woven combination of silk and cotton, and a wear-resistant coating matter fastened to one face

75

80

85

90

95

100

110

115

120

125

130

of said uninked absorbent silk and cotton combination, and having one face of said uninked silk and cotton combination, only, coated with said wear-resisting matter and 5 material, and said wear-resisting material being unfit to transfer ink therethrough to the type faces and it does not impregnate and does not fill up the interstices of said silk and cotton combination, and said coating being 10 distinguished by the fact that no adhesive and no liquid cement and no foreign material is between it and said silk and cotton combination, and when said coating is thoroughly dry, it is of such character it can- 15 not injure said silk and cotton and cannot injure said ink which is later applied to said silk and cotton and said ink fills the interstices of said silk and cotton combination.

36. An ink transfer member comprising 20 a compact, closely woven, tight uninked base material composed of a combination of absorbent silk and cotton, ink, and a wear-resisting coating, said coating being unfit for transferring ink therethru and when 25 thoroughly dry taking and retaining on its surface at least one ingredient of a typewriter ribbon ink, and said coating being on the surface of the side towards the type and on said surface only of said base and said coating 30 does not impregnate said base but said base is impregnated with ink and the interstices of said silk and cotton combination material 35 are filled with ink.

37. An ink transfer member comprising 40 an uninked base material and a coating fastened securely to said uninked base material on the side to be struck by the type, and ink, and having the edges of the uninked base material impregnated with a material impervi- 45 ous to ink, and having no coating on the face towards the writing surface, and the coating on the type side is unfit for the passage of ink through to the type faces, and the base is im- 50 pregnated with ink and the interstices of the base are full of ink and the coating does not 55 impregnate the base and does not materially impair the ink absorbing capacity of said base material.

38. An ink transfer member comprising 60 an uninked base material, a coating fastened securely to said uninked base material on the face to be struck by the type and towards the type, and ink, and having no coating towards the writing surface, and said coating is of 65 such character that it is not possible to screen ink through same and it is possible to trans- 70 fer ink impressions to a writing surface from the uncoated face and said member car- 75 rying ink and nothing else on the uncoated face, and the base being impregnated with 80 ink and the interstices of said base being full 85 of ink and said coating does not materially 90 reduce the absorbency of said base material 95 and said coating extends the life of the base.

65 39. A transfer member of the character

described, comprising ink, an uninked base material and a coating on one face of said uninked base material and said coated face being less ink absorbent than the uncoated face, and inked on both faces, and said trans- 70 fer member being distinguished by the fact that it is not possible to transfer ink im- 75 pressions except from the uncoated face and said base being impregnated with ink and the interstices of the said base being filled 80 with ink, said inking being an operation per- 85 formed after the application of said coating to the uninked base material, and said mem- 90 ber has less ink on the coated face than it has 95 on the face towards the writing surface.

In testimony whereof I affix n.y signature.  
GEORGE E. PELTON.

70

75

80

85

90

95

100

105

110

115

120

125

130